

# UNITED STATES PATENT OFFICE.

WILLIAM RINTOUL AND DONALD CROSS, OF STEVENSTON, SCOTLAND, ASSIGNEES TO  
NOBEL'S EXPLOSIVES COMPANY LIMITED, OF STEVENSTON, SCOTLAND.

## EXPLOSIVE.

1,306,440.

Specification of Letters Patent. Patented June 10, 1919.

No drawing.

Application filed September 24, 1917. Serial No. 192,964.

To all whom it may concern:

Be it known that we, WILLIAM RINTOUL and DONALD Cross, both subjects of the King of Great Britain and Ireland, and residing at Ardeer Factory, Stevenston, Ayrshire, Scotland, have invented certain new and useful Improvements in Explosives, of which the following is a specification.

This invention relates to improvements in the manufacture of blasting explosives containing nitroglycerin and gelatinized nitrocellulose.

In this class of explosive it has been proposed to employ aromatic nitro-bodies soluble in nitro-glycerin as components for the purpose of making the so-called "non-freezing explosives".

It has also been proposed to promote the solubility upon which gelatinization depends by the addition of a small quantity of substances such as the acetic ethers of glycerin ethyl, and methyl, acetic acid, a mixture of alcohol and ether, acetone, nitrobenzol, dinitro-benzol, the nitrates of methyl, and ethyl and other analogous substances.

It has thus been proposed to employ a proportion of the substance depending on its nature but as a rule about 10% of the weight of the nitroglycerin was indicated. Further in such connection it was stated that by the use of heat the quantity to be used could be reduced to 2% or even less.

Notwithstanding these proposals such "non-freezing" and other blasting explosives of this type have hitherto been universally made by mixing the nitrocellulose and the nitroglycerin and the component adapted to give non-freezing properties, adding the other ingredients, if any, and completing the mixing by stirring while heated by a water jacket maintained at an elevated temperature of for instance 60 to 70° C. The high temperature of mixing has hitherto been considered necessary in order to effect the gelatinization of the nitrocellulose and the dangerous nature of the manufacture of such explosives is largely due to this use of a high temperature during gelatinization, which also considerably increases the cost of manufacture.

Now we have discovered that aromatic nitro-bodies soluble in nitroglycerin, when

dissolved in certain small proportions in the nitroglycerin have the property of gelatinizing completely in the cold all classes of nitrocellulose from the soluble variety up to gun-cotton containing 13% nitrogen, and that the gelatinization so carried out takes place more rapidly than when nitroglycerin alone is used at a temperature of from 60 to 70° C.

This invention therefore consists in employing as a gelatinizing accelerant along with nitroglycerin and dissolved therein, a small proportion of the order of 0.1 to 1% calculated on the nitroglycerin, of an aromatic nitro-body, and in effecting the gelatinization of the nitrocellulose of the blasting explosive thereby without elevation of temperature.

In carrying this invention into effect in one form by way of example, we employ a small quantity of from 0.1% to 1% calculated on the nitroglycerin of one of the following aromatic nitro-bodies soluble in nitroglycerin:—

Mono, di or tri-nitro-toluene;

Mono-nitro-naphthalene;

Di-nitro-benzene;

Nitro-xylenes; or

Mixtures of these bodies;

and dissolve them in the nitroglycerin of the blasting composition. We then stir the nitrocellulose into this nitroglycerin solution, and the other ingredients, if any, and complete the mixing in the usual manner, but without elevation of temperature. A good blasting explosive is thus prepared in all respects equal to the corresponding product prepared by the method of hot gelatinization, while the risks attendant on the use of the latter process are avoided, the output of a given plant is increased, and a marked reduction in the cost of manufacture is effected.

The following are the compositions of typical examples of explosives made as above according to this invention:—

### I. Modified blasting gelatin.

|                        |       |     |
|------------------------|-------|-----|
| Nitroglycerin          | 89.8% |     |
| Soluble nitrocellulose | 8.7%  |     |
| Liquid trinitrotoluene | .9%   | 105 |
| Calcium carbonate      | 0.6%  |     |

11. *Modified gelignite.*

|   |                        |       |
|---|------------------------|-------|
| 5 | Nitroglycerin          | 0.5%  |
|   | Soluble nitrocellulose | 3.8%  |
|   | Potassium nitrate      | 27.6% |
|   | Woodmeal               | 7.2%  |
|   | Liquid trinitrotoluene | .6%   |
|   | Calcium carbonate      | 0.3%  |

10 We find that while ordinary blasting gelatin of the following composition:

|    |               |        |
|----|---------------|--------|
| 15 | Nitroglycerin | 90.6%  |
|    | Nitro-cotton  | 8.8%   |
|    | Chalk         | 0.6%   |
|    |               | 100.0% |

20 prepared according to the service method at 60-70°C. requires about 75 minutes for gelatinization, a corresponding blasting gelatin with an accelerator as in Example I above requires only about 45 minutes for gelatinization at normal temperature. Again, while ordinary gelignite of the following composition:

|    |                   |        |
|----|-------------------|--------|
| 25 | Nitroglycerin     | 61.1%  |
|    | Nitro-cotton      | 3.8%   |
|    | Woodmeal          | 7.2%   |
|    | Potassium nitrate | 27.6%  |
|    | Chalk             | 0.3%   |
|    |                   | 100.0% |

30 prepared according to the service method at 60-70°C. requires about 75 minutes, a corresponding gelignite with an accelerator as in Example II above requires only about 55

minutes for gelatinization at normal temperature.

35 The expression "aromatic nitro-body" is used in the claims to include either a single aromatic nitro-compound capable of acting as an accelerator, or a mixture of two or more such bodies, said mixture having accelerating properties.

40 Having now described our invention, what we claim as new and desire to secure by Letters Patent is:—

45 1. The manufacture of nitroglycerin nitrocellulose blasting explosives containing more than 50% nitroglycerin by dissolving in the nitroglycerin an aromatic nitro-body in small proportion of the order of 0.1 to 1% calculated on the nitroglycerin, and effecting the gelatinization of the nitrocellulose thereby without elevation of temperature, substantially as described.

50 2. A cold-gelatinized blasting explosive comprising nitroglycerin, nitrocellulose, and a nitro-aromatic accelerator for the gelatinization in amount not exceeding substantially one per cent. calculated on the nitroglycerin content.

55 3. A cold-gelatinized nitroglycerin nitrocellulose blasting explosive containing more than 50% nitroglycerin and a small proportion of the order of 0.1 to 1 per cent, calculated on the nitroglycerin, of a gelatinizing accelerator consisting of an aromatic nitro-body.

60 In testimony whereof we have signed our names to this specification.

70 WILLIAM RINTOUL.  
DONALD CROSS.